

April 2, 1940.

J. KORPIUN

2,196,018

CARTRIDGE CASE PROVIDED WITH A NONMETALLIC SURFACE

Filed Aug. 3, 1936



INVENTOR.

Joachim Korpium

BY

*St. C. B.*

ATTORNEY.

## UNITED STATES PATENT OFFICE

2,196,018

CARTRIDGE CASE PROVIDED WITH A  
NONMETALLIC SURFACEJoachim Korpian, Berlin-Grunewald, Germany,  
assignor to Schering Aktiengesellschaft, Berlin,  
Germany, a corporation of GermanyApplication August 3, 1936, Serial No. 94,055  
In Germany August 3, 1935

7 Claims. (Cl. 102—16)

This invention refers to cartridge cases, and more especially to cartridge cases provided with a nonmetallic surface.

With cartridge cases for rifles, guns and the like, made of brass, especially with those of larger calibers and when the barrels have become hot, the danger exists, that they are welded together with the gun barrel whereby in most of the cases the latter becomes completely useless.

It should be possible to avoid or at least to substantially diminish said danger when using a raw material for making the cartridge cases the melting point of which is sufficiently high. Raw materials with a melting point that is high enough for this purpose, however, cannot be employed in making cartridge cases on account of their high costs and the fact that in general they can only be worked with difficulty.

By the present invention a new way to overcome said difficulties has been found, that consists in providing suitable layers of separation between the cartridge case and the wall of the barrel, said layers excluding metallic contact between these two parts even when they are in a highly heated condition. Such layers of separation may consist, for instance, of oxides or mixtures of oxides that have been produced upon the cartridge itself by artificial means. Preferably the melting point of the layer of separation shall be higher than that of at least one metal component of the alloy that might be formed on welding of the cartridge case and the wall of the barrel. The best results are achieved when the layer of separation is artificially formed from the basic material of the cartridge case itself.

The use of this inventive idea proved to be of special advantage when employing aluminum as raw material for the cartridge cases. A uniform aluminum oxide layer of a high melting point as it is artificially produced upon the aluminum by oxidation, is an especially suitable layer of separation for preventing the welding together as well as the formation of an alloy between the highly heated metals; thereby the danger of the cartridge case becoming welded together with the barrel is eliminated.

The oxide layers for this purpose may be applied to the aluminum either by chemical means, for instance, by boiling the cartridge case with oxidizing solutions, such as chromate solutions, or better and more efficiently by electrolytic oxidation of the aluminum. The thickness of said layers is in general between 0.1 and 30  $\mu$  but, of course, may even be greater.

According to the electrolytic method the ox-

idation may be carried out, for instance, in a simple and convenient manner in sulfuric acid or oxalic acid solution by means of alternating or direct current. However, the use of baths of this type for carrying out the oxidation is not necessary; for, other electrolytic baths that are suitable to produce oxide layers on aluminum by means of direct or alternating current may be employed likewise.

Besides the special property of preventing the burning together of cartridge case and barrel, such cartridge cases made of superficially oxidized aluminum have the further advantage that they possess a hard and smooth surface and hence, do not corrode even on storing the same in a moist atmosphere. Thus, such cartridge cases enable proper working of the firearms under all conditions in contrast with cartridge cases of brass on the surface of which on storing in a moist atmosphere verdigris and the like is formed, causing their diameter to become enlarged over the admissible tolerance on account of the larger volume of the verdigris so that the charging of the firearm is impeded or other disturbances may take place. Furthermore it might be mentioned that the use of aluminum for cartridge cases means a considerable saving in weight.

Instead of the oxidic layer of separation on aluminum cartridge cases there may be used layers composed of other material, such as a fluoride or phosphate or the like layer.

Instead of aluminum also its alloys may be employed as raw material for the cartridge case, whereby upon oxidation a mixture of the oxides of the metals in said alloys is produced.

Of course, many other changes and variations may be made by those skilled in the art in accordance with the principles set forth herein and in the claims annexed hereto.

What I claim is:

1. A cartridge case comprising an aluminum containing case adapted for use in a gun barrel and an aluminum oxide layer thereon, said layer produced by electrolytic oxidation of said aluminum cartridge case, said layer being integral with said case, whereby fusion of said case and welding to said gun barrel in the firing of cartridges is prevented even under conditions of high temperatures.

2. A cartridge case comprising an aluminum containing case adapted for use in a gun barrel and an aluminum oxide layer thereon, said layer being produced by electrolytic oxidation of said aluminum cartridge case by means of a sulphuric acid bath, said layer being integral with

said case, whereby fusion of said case and welding to said gun barrel in the firing of cartridges is prevented under conditions of high temperatures.

3. A cartridge case comprising an aluminum containing case adapted for use in a gun barrel and a layer thereon, said layer selected from the group of materials consisting of artificially produced aluminum oxide, aluminum fluoride and aluminum phosphate, said layer being integral with said case, whereby fusion of said case and welding to said gun barrel in the firing of cartridges is prevented even under conditions of high temperatures, the thickness of said oxide layer being considerably greater than that formed by natural atmospheric oxidation of aluminum.

4. A cartridge case comprising a case consisting of an aluminum alloy adapted for use in a gun barrel, and a layer thereon, selected from the group of materials consisting of artificially produced aluminum oxide, aluminum fluoride and aluminum phosphate, said layer being integral with said case, whereby fusion of said case and welding to said gun barrel in the firing of cartridges is prevented even under conditions of high temperatures, the thickness of said oxide layer being considerably greater than that formed by natural atmospheric oxidation of aluminum.

5. A cartridge case comprising a case consisting essentially of aluminum and adapted for use in a gun barrel and a firmly adherent surface layer of an aluminum compound thereon, said surface

layer excluding a welding of the cartridge case and the barrel wall of firearms, having a high melting point and being artificially produced from the material of the cartridge case by reaction with suitable substances to provide a layer taken from the class consisting of oxide, fluoride and phosphate.

6. A cartridge case comprising a case consisting essentially of aluminum and adapted for use in a gun barrel and a firmly adherent surface layer of an aluminum compound thereon, said surface layer excluding a welding of the cartridge case and the barrel wall of firearms, having a high melting point, comprising aluminum oxide and being artificially produced from the material of the cartridge case by reaction with suitable substances to provide a layer taken from the class consisting of oxide, fluoride and phosphate.

7. A cartridge case adapted for use in a gun barrel comprising an aluminum containing case and a layer containing aluminum oxide thereon, said layer being artificially produced from the material of the cartridge case, being integral therewith and having a thickness of 0.1 to 30  $\mu$ , whereby fusion of said case and welding to said gun barrel in the firing of cartridges is prevented even under conditions of high temperatures, the thickness of said oxide layer being considerably greater than that formed by natural atmospheric oxidation of aluminum.

JOACHIM KORPIUN.